

## UNITED STATES PATENT OFFICE

2,524,825

## METAL CLEANING COMPOSITION

Arthur C. Pabst, Douglaston, N. Y., and Eleanor S. Salmon, New York, N. Y., assignors to Secony-Vacuum Oil Company, Incorporated, a corporation of New York

No Drawing. Application September 14, 1945,  
Serial No. 616,478

3 Claims. (Cl. 252—143)

1

This invention relates to improved metal cleaning compositions and their uses. It is particularly directed to metal cleaning compositions capable of removing rust, scale, grease and other deposits from metal surfaces.

One of the main uses for such a composition is in the cleaning of water cooling systems such as are used in internal combustion engines. Such systems gradually become fouled during use and unless periodically shut down and cleaned, the water jackets and radiators become coated with deposits which interfere with the heat transfer and in severe cases may be plugged to a point of complete stoppage of coolant circulation. The composition of the deposits may vary depending upon the construction materials of the coolant system. Such metals as solder, copper, zinc, lead and iron may be used in one form or another and, of these, iron in its various modifications is the chief component. Grease may enter the cooling system from grease packed water pumps and oil or oxidized hydrocarbons may enter from "blow-by" from the combustion chamber or from other sources. Certain other foreign deposits may be introduced with the coolant especially when it is water. A common component of the fouling deposits is iron oxide cemented fast to the metal surface by adsorbed or oxidized oil. Such a scale especially when covered with a coating of grease or oil is very difficult to remove.

Similar conditions prevail and similar contaminants consisting of oxidized metal and oily substances are usually present on the surfaces of machine parts which are to be cleaned in shops. The cleaning operations usually comprise degreasing, pickling and de-rusting.

Cleaning compositions used at present for automotive cooling systems may be generally classified under one of three types. One type consists of an aqueous solution of an alkaline salt such as washing soda, trisodium phosphate, etc. This type acts very slowly on rust and scale so that only small amounts of the deposits are removed in the time normally given the radiator flushing. Moreover it removes very little of the oil or grease deposits. A second type of cleaner consists of an alkaline emulsion of hydrocarbon and other organic solvents. This type will remove the oil and grease deposits fairly satisfactorily but will remove only very small amounts of rust and scale deposit; consequently, the system is not entirely cleaned. The third type of cleaner consists of

2

aqueous solutions of acids or acid salts, such as hydrochloric and oxalic acids and sodium bisulfate. This type is very effective in removing rust and scale but will remove very little grease or oil deposit. Moreover, the acid type cleaner is highly corrosive and requires a "follow-up" flush with an alkali to stop the action of the acid. This is not always satisfactory in entirely avoiding corrosion as it is often difficult to obtain complete acid neutralization.

A major object of this invention is the provision of a new and novel cleaning composition which is capable of removing rust, scale and oily deposits.

A further object of this invention is the provision of a cleaning composition which will rapidly remove rust and scale deposits from metal surfaces without causing rapid "after corrosion" of the metal surface.

Another object is the provision of a rapid method for cleaning metal surfaces and cooling systems which will not cause considerable surface corrosion. These and other objects will become apparent from the more detailed description of the invention following hereinafter.

We have now discovered that certain oil-in-acid solution type emulsions will rapidly remove rust and scale from metal surfaces and at the same time dissolve and emulsify any oil and grease present. Tests also indicate that the product has remarkable properties in inhibiting corrosion so that it is unnecessary to follow up with an alkaline wash. In other words, the product offers the main advantages of each of the types of common radiator flushes without their disadvantages and failings.

These emulsions consist of a dispersed phase of an emulsifiable organic water-insoluble material and a continuous phase of a strong aqueous solution of hydrochloric acid, said solution being of the order of 4 pH or lower, and a specific emulsifying agent capable of producing emulsions sufficiently stable both for long shelf storage prior to use and for subsequent dilution if desired at the time of use while still forming a stable emulsion.

The aqueous phase as pointed out above is a strong solution of hydrochloric acid, sufficiently strong in the base composition to permit considerable dilution and still give a composition of sufficient strength for the ultimate cleaning purpose, that is the solution of scale, rust, sludge, and the like when applied in cleaning. The dispersed phase may consist either of hydro-

carbon solvents or of halogenated hydrocarbon solvents or mixtures thereof; exemplary are kerosene and orthodichlorbenzene. Halogenated hydrocarbons either alone or in admixture with straight hydrocarbons are particularly desirable as they tend to form stable emulsions more readily. This is probably because of their high specific gravity. Preferably, such hydrocarbons and halogenated hydrocarbons should boil above about 160° F. in order to prevent loss thereof by evaporation during use.

The emulsifier to be used is one capable of giving either a completely stable emulsion or a readily redispersable product when the emulsion is stored over long periods of time, for example as shelf goods. One such emulsifier is polyethylene-glycol mono iso-octyl phenyl ether. Another such emulsifier is 1-hydroxyethyl 2-heptadecenyl glyoxalidine. A preferred form of composition is one which contains both of these emulsifiers in admixture.

The following examples will illustrate the type of emulsions made and used according to this invention:

| Emulsion No.                                      | I    | II              | III             | IV              | V               |
|---------------------------------------------------|------|-----------------|-----------------|-----------------|-----------------|
| Constituents                                      |      |                 |                 |                 |                 |
| Orthodichlorbenzene                               |      | Weight per cent | Weight per cent | Weight per cent | Weight per cent |
|                                                   | 20.0 | 20.0            | 20.0            | 39.5            | 19.5            |
| Kerosene                                          |      | 20.0            | 19.5            | 19.5            | 19.0            |
| Concentrated HCl (38%)                            |      | 58.5            | 27.0            | 27.0            | 59.0            |
| 1-hydroxyethyl, 2-heptadecenyl glyoxalidine       |      | 1.5             | 1.5             |                 | 1.5             |
| Polyethylene-glycol, mono iso-octyl, phenyl ether |      |                 |                 | 5.0             |                 |
| Water                                             |      |                 |                 |                 | 1.0             |
|                                                   |      | 32.0            | 32.0            | 28.5            |                 |

These emulsions are prepared by dissolving the emulsifier in one of the phases, generally the one in which the emulsifier is most soluble, and then adding the other liquid phase while stirring the liquid with a higher speed mixer. The hydrocarbon emulsion in aqueous acid thus formed may be further diluted with water, if desired. Either the cationic emulsifier 1-hydroxyethyl 2-heptadecenyl glyoxalidine or the non-ionic emulsifier, polyethyleneglycol mono iso-octyl phenyl ether are soluble in the oil phase and may be dissolved therein and the acid then added. Moreover, the former emulsifier is also soluble in aqueous acid solution, so that it may first be dissolved therein and the oil phase added with mixing. The desirable amount of emulsifier to be used may vary between 0.1% to 5.0% by weight of the emulsion. In use the prepared emulsion may be added to the cooling system or to a circulating bath in concentrations controlled to provide the desired cleaning rate. Thus, for example, such prepared emulsions as shown in the above table may be added to water in a cooling system in concentrations of 5% emulsion and upwards. In any event the pH value of the liquid circulated in the cleaning system should be below 4.0. It will be noted that in Emulsions II and III in the above table, the concentrations of the HCl in the continuous phase is 17.4 percent by weight while in Emulsion V the concentration of HCl in the continuous phase is 38 percent by weight.

After the emulsion is added to the cooling system or cleaning bath, it is heated either by a heater or by starting the engine involved and the heated emulsion is circulated. After about 20 to 30 minutes of circulation, the system is drained and flushed by filling with water and running the

engine until warm. The water is then drained and the system refilled with cooling water. After such a treatment, the metal surfaces of the cooling system are thoroughly clean of rust, scale, water deposits and grease. When the cleaning solution is used for cleaning metal parts or tools, the parts or tools are placed in a bath of the emulsion for a set period, then removed and rinsed in clean water. No neutralizing chemicals need be added to the rinsing water to prevent corrosion of the metal cleaned.

In addition to the practical tests on automobile cooling systems, as described hereinabove, laboratory tests were also made to establish the relative cleaning efficiencies of these novel emulsions and of certain cleaning composition used commercially heretofore. Rusted steel plates were immersed in the boiling solutions in concentrations recommended by the respective manufacturers, and the time required for completion of cleaning was taken as a measure of efficiency. The after corrosion of the metal was particularly noted.

| Concentration of Active Acid or Salt in Cleaning Bath | Time, in minutes, to complete cleaning | After-corrosion in four days | 25                     |
|-------------------------------------------------------|----------------------------------------|------------------------------|------------------------|
|                                                       |                                        |                              | Gm./liter              |
| 30                                                    | 30                                     | noticeable.                  | Oxalic acid type       |
|                                                       | 30                                     | Do.                          | Sodium bisulfate type  |
|                                                       | 7                                      | strong.                      | Hydrochloric acid type |
|                                                       | 7                                      | none.                        | Emulsion II (1:9)      |

It will be apparent from the above that the emulsions of this invention have substantially the same rust removing power as strong acid type commercial cleaning compositions while at the same time protecting the metal surface cleaned from after corrosion. Moreover, the emulsions have a far greater grease and oil removing power than the acid or acid salt type cleaning compositions. The stable hydrocarbon-in-acidic-solution emulsion permits a uniformity of hydrocarbon distribution throughout the cleaning solution so that it may perform its function uniformly over the entire surface of the metal to be cleaned.

To further prove that the emulsion type cleaning compositions of this invention are less corrosive on the metal surfaces or cooling systems being cleaned, even while being used, a number of uniform strips of the metals commonly encountered in cooling systems were immersed in several different cleaning liquids for a period of 24 hours and the corrosion loss was then measured.

| Concentration of Active Acid or Salt in Cleaning Bath | Corrosion loss at 160° F. in 24 hrs. |        |
|-------------------------------------------------------|--------------------------------------|--------|
|                                                       | Iron                                 | Solder |
| 60                                                    |                                      |        |
|                                                       | Gm./liter                            | Mg.    |
| 65                                                    | 20                                   | 146    |
|                                                       | 23                                   | 3,140  |
|                                                       | 10                                   | 52     |
|                                                       | 20                                   | 300    |
|                                                       |                                      | Mg.    |
|                                                       |                                      | 33.5   |
|                                                       |                                      | 748    |
|                                                       |                                      | 19.1   |
|                                                       |                                      | 21.1   |

It should be understood that the specific examples of the emulsion type cleaning composition and of their application as given hereinabove are intended merely as exemplary and are not to be construed as limiting the scope of this invention thereto. These compositions present a very considerable and useful stability over related

compositions known to the prior art as may be seen from the following data.

ACID EMULSIONS  
*Metal cleaning compositions*

|                                                | #1    | #2    | #3    | #4    | #5    | #6    | #7    |
|------------------------------------------------|-------|-------|-------|-------|-------|-------|-------|
| 6 Normal HCl                                   | 59.0  | 59.0  | 59.0  | 59.0  | 59.0  | 59.0  | 59.0  |
| Hydrocarbon solvents of kerosene boiling range | 19.0  | 19.5  | 17.5  | 19.5  | 19.5  | 19.5  | 19.5  |
| Orthodichlorbenzene                            | 19.5  | 20.0  | 18.5  | 20.0  | 20.0  | 20.0  | 20.0  |
| 1-hydroxyethyl, 2-heptadecenyl, glyoxalidine   | 1.5   |       |       |       |       |       |       |
| Polyethylene-glycol monoiso-octyl phenyl ether | 1.0   |       |       |       |       |       |       |
| Sodium Lauryl Sulphate                         |       |       |       |       |       |       |       |
| Gum Tragacanth                                 |       | 1.5   | 5.0   | 1.5   |       |       |       |
| Polyethylene Glycol Monoleate 600              |       |       |       |       | 1.5   |       |       |
| Polyethylene Glycol Dioleate 600               |       |       |       |       |       | 1.5   |       |
| Polyethylene Glycol Oleate 400 L               |       |       |       |       |       |       | 1.5   |
|                                                | 100.0 | 100.0 | 100.0 | 100.0 | 100.0 | 100.0 | 100.0 |
|                                                | (1)   | (2)   | (3)   | (4)   | (5)   | (6)   | (7)   |

## PROPERTIES OF THE EMULSIONS

<sup>1</sup> Emulsion stable for 1 day. Separates into 2 emulsion layers in 3 days. Redispersed by simple shaking after 6 months. Forms stable emulsion when diluted, can be boiled.

<sup>2</sup> Ex. 2: Unstable. Total separation and no redispersion after 5-10 minutes.

<sup>3</sup> Ex. 3: Unstable. Separation begins within 5-10 minutes. Total separation and no redispersion after 12 hours.

<sup>4</sup> Ex. 4: No emulsion. Water phase too thick. Cannot be dispersed.

<sup>5</sup> Ex. 5: Stable for 1 day. Separates into 2 clear phases in 3 days and cannot be redispersed by vigorous shaking. Cannot be diluted. Forms no emulsion in water.

<sup>6</sup> Ex. 6: Stable for 1 day. Separates into 2 clear phases in 3 days and cannot be redispersed by vigorous shaking. Cannot be diluted. Forms no emulsion in water.

<sup>7</sup> Ex. 7: Stable for 1 day. Separates into 2 clear phases in 3 days and cannot be redispersed by vigorous shaking. Cannot be diluted. Forms no emulsion in water.

It is noticeable that while emulsion number 1, which is an emulsion of the preferred type herein disclosed has about the same stability as a complete emulsion, as others, particularly compositions 5, 6 and 7, when separation does occur, the material still remains as two emulsion phases rather than two clear phases, even after 6 months' storage. The material by simple shaking may be redispersed to form an emulsion. Further, that the material of column 1 can be diluted with water still forming a stable emulsion and that this dilute emulsion can be boiled thus demonstrating a very considerable difference in nature between the materials herein disclosed and somewhat related materials common in the art.

This case is a continuation-in-part of our application Serial No. 562,902 filed November 10, 1944, now abandoned.

We claim:

1. A metal cleaning composition in the form of an oil-in-water type emulsion which comprises: a dispersed phase of a substantially water-insoluble solvent selected from the group consisting of orthodichlorbenzene, and mixtures of orthodichlorbenzene and hydrocarbon solvents boiling in the kerosene boiling range, a continuous phase of a strong aqueous solution of hydrochloric acid in which the concentration of HCl is within the range about 17.4 to 38 percent by weight and about 0.1 percent to about 5.0 percent by weight of the emulsion of 1-hydroxyethyl 2-heptadecenyl glyoxalidine as an emulsifier.

2. A metal cleaning fluid in the form of an oil-in-water type emulsion which comprises: a dispersed phase of a mixture of kerosene and ortho-

6 dichlorbenzene, a continuous phase of a strong aqueous solution of hydrochloric acid in which

the concentration of HCl is within the range about 17.4 to 38.0 percent by weight, and between about 0.1 percent and about 5.0 percent by weight of the emulsion of 1-hydroxyethyl 2-heptadecenyl glyoxalidine as an emulsifier.

3. A metal cleaning fluid for cleaning rust, scale and grease from the surface of fluid-circulated cooling system, in the form of an oil-in-water type emulsion which comprises a dispersed phase of a mixture of kerosene and orthodichlorbenzene, a continuous phase of a hydrochloric acid aqueous solution, and about 0.1 percent to about 5.0 percent by weight of the emulsion of 1-hydroxyethyl 2-heptadecenyl glyoxalidine as an emulsifier, the concentrations of HCl in said emulsion amounting to at least about 10 grams per liter.

ARTHUR C. PABST.  
ELEANOR S. SALMON.

## REFERENCES CITED

50 The following references are of record in the file of this patent:

## UNITED STATES PATENTS

| Number    | Name      | Date          |
|-----------|-----------|---------------|
| 2,036,848 | Amthor    | Apr. 7, 1936  |
| 2,261,700 | Ryznar    | Nov. 4, 1941  |
| 2,269,529 | Goldsmith | Jan. 13, 1942 |
| 2,302,697 | Katzman   | Nov. 24, 1942 |
| 2,396,776 | Douty     | Mar. 19, 1946 |

## OTHER REFERENCES

Bennett: Chemical Formulary, vol. 2 (1935), page 73.